# EUROPEAN PATENT APPLICATION

(11) **EP 1 752 519 A1**
(43) Date of publication of application: **14.02.2007**
(21) Application number: 05739172.4
(22) Date of filing: 28.04.2005
(51) Int. Cl.: C10M 171/00, C10M 169/04, C10M 177/00, F04B 27/08, F04B 39/00, C10M 103/02, C10M 103/06, C10M 107/38, C10M 145/18, C10M 149/14, C10N 10/12, C10N 30/06, C10N 40/02, C10N 50/08, C10N 70/00

(54) **SLIDE MEMBER AND METHOD OF PRODUCING SLIDE MEMBER**

(30) Priority: 27.05.2004 JP 2004157825
(71) Applicant: KABUSHIKI KAISHA TOYOTA JIDOSHOKKI, Kariya-shi, Aichi 448-8671 (JP)
(72) Inventor: MURASE, Hitotoshi, c/o K.K. TOYOTA JIDOSHOKKI, Kariya-shi, Aichi 4488671 (JP); SHIMO, Toshihisa, c/o K.K. TOYOTA JIDOSHOKKI, Kariya-shi, Aichi 4488671 (JP)
(74) Representative: TBK-Patent
(86) International application number: PCT/JP2005/008582
(87) International publication number: WO 2005/116175

(57) **Abstract**

A slide member of the present invention is a slide member having a substrate (10) made of a metal; and a sliding layer (20) of a resinous powder being sintered integrally on at least one of the surfaces of the substrate (10), and is **characterized in that** it includes a solid-lubricant powder in the sliding layer (20). Further, it can be one having an intermediate layer, which intervenes between the substrate (10) and the sliding layer (20), and which is composed of a metal differing from that of the substrate (10). The slide member of the present invention is such that the adhesiveness is high, and has good sliding characteristics.

Moreover, a production process of the present invention for a slide member is **characterized in that** it has: a laminating step of forming a powdery sliding layer, which is composed of a resinous powder and a solid-lubricant powder at least, on at least one of the surfaces of a substrate layer, which is composed of a metal; and a sintering step of sintering the substrate layer with the powdery sliding layer integrally. In accordance with this production process, it is possible to make a slide member, which has the substrate (10) and the sliding layer (20) at least. In accordance with the production process of the present invention for a slide member, it is possible to produce a slide member whose adhesiveness is high and which has good sliding characteristics.

## Description

### TECHNICAL FIELD

The present invention relates to a slide member, which is used for the sliding portion of various apparatuses, and a production process for the same.

### BACKGROUND ART

A slide member, which is used for a compressor, and the like, comprises a substrate made of a metal, and a sliding layer made of a resin, which is formed on its sliding surface; and the sliding performance of the slide member is improved by means of the sliding layer. In many cases, the sliding layer is formed by means of coating a film made of a resin; for example, in Japanese Unexamined Patent Publication (KOKAI) No. 11-13, 638, a sliding layer is obtained via drying and calcining after a thermosetting resin, which is solved in a solvent, is applied onto a substrate made of a metal by means of spray coating, and so forth.

When forming a sliding layer by means of coating, since drying and calcining are carried out after coating, the number of processing steps has become many. In particular, when forming a sliding layer comprising a plurality of layers, since the aforementioned processing steps are carried out repeatedly, the number of processing steps has become many furthermore. Moreover, for the selection of a solvent in which a resin is solved and the disposal for the same, it is necessary to consider the safety and environmental issues.

As one of the forming processes for the sliding layer, which substitutes for coating, a sintering method can be thought of. However, according to Comparative Example No. 1 of Japanese Patent Unexamined Publication (KOKAI) Gazette No. 9-131,828, when a layer, which is composed of an aluminum powder alone, and a layer, which is composed of a polyimide powder alone, are laminated and are then sintered, they come off easily at the interface between both of the components. Accordingly, in Japanese Patent Unexamined Publication (KOKAI) Gazette No. 9-131,828, the adhesiveness between both of the layers is secured by means of forming a layer, which includes a metal and a resin simultaneously, between the layer, which is composed of a metal alone, and a layer, which is composed of a resin alone. Namely, it is not easy to form a sliding layer, which is made of a resin, on a substrate, which is made of a metal, by means of sintering.

### DISCLOSURE OF THE INVENTION

In view of the aforementioned circumstances, the present inventors found out a noble construction, which can secure the adhesiveness between a substrate layer and a sliding layer even by means of sintering. Namely, the present invention is a slide member, which can be obtained by means of sintering, and is such that it is an object to provide a slide member, whose adhesiveness between a substrate and a sliding layer is high and which is suitable for sliding portions, and a production process for the slide member.

A slide member of the present invention, which solves the aforementioned problems, is a slide member having a substrate made of a metal; and a sliding layer of a resinous powder being sintered integrally on at least one of the surfaces of the substrate, and is characterized in that it includes a solid-lubricant powder in said sliding layer.

By means of the fact that a solid-lubricant powder is included in the sliding layer, the difference between the linear expansion coefficients of the substrate and sliding layer becomes smaller. As a result, it is possible to secure the adhesiveness between the substrate made of a metal and the sliding layer made of a resin, adhesiveness which has not been obtainable by sintering so far. Further, since the sliding layer is formed by means of solidifying after the resinous powder is melted by means of sintering, it is good in terms of the adhesiveness to the substrate. Moreover, when it is sintered while being pressurized, since the resinous powder melts and then solidifies in such a state that it is pressurized, it is furthermore good in terms of the adhesiveness.

Said substrate can preferably be a bulk body, or a sintered body, which is composed of a metal powder being sintered integrally with said sliding layer. Here, "bulk" means "mass," and is usually referred to those other than thin films and wire rods. Namely, in the substrate being a bulk body, sintered bodies, which are composed of metal powders, not being those which are sintered integrally with the sliding layer, in other words sintered bodies which are formed by means of sintering in advance before sintering the sliding layer are included as well, in addition to metallic members which are processed by means of casting, and the like.

Said sliding layer can preferably be a functionally-gradient-material layer in which a volume fraction of said solid-lubricant powder on its substrate side is lower than on an opposite substrate side. By mean of adapting the sliding layer to a functionally-gradient-material layer, it is possible to secure the adhesiveness to the substrate while providing the opposite substrate side with good sliding characteristics. In this instance, said functionally-gradient-material layer can preferably be a layer in which the proportion of said solid-lubricant powder changes continuously or stepwise from said substrate side to said opposite substrate side.

Further, it can preferably have an intermediate layer. By means of disposing an intermediate layer, even when such an instance occurs that the sliding layer is damaged during the slide member's service, since it can keep sliding to adapt the intermediate layer to a sliding surface, the reliability as a slide member improves. In this instance, said intermediate layer can preferably be an intermediate sintered-body layer, which is composed of a metal powder being sintered integrally with said substrate and said sliding layer.

Moreover, a production process of the present invention for a slide member is characterized in that it has: a laminating step of forming a powdery sliding layer, which is composed of a resinous powder and a solid-lubricant powder at least, on at least one of the surfaces of a substrate layer, which is composed of a metal; and a sintering step of sintering the substrate layer with the powdery sliding layer integrally.

Since the substrate layer and powdery sliding layer, which are formed in the laminating step, are sintered integrally in the sintering step, it is possible to form a slide member through the reduced number of steps. Moreover, since the powdery sliding layer includes a solid-lubricant powder, the difference between the linear expansion coefficients of the after-sintering substrate layer and powdery sliding layer becomes smaller. As a result, no coming-off occurs from the interface between the after-sintering substrate layer and powdery sliding layer. Further, since sintering is used, no solvent, which is essential in coating, is needed; and, moreover, even when being a sliding layer which is composed of a resinous powder being less likely to solve into a solvent, the formation is made possible. Moreover, by means of forming the substrate layer and powdery slide member with compression in the laminating step, or sintering while pressurizing them, a slide member, which is good in terms of the adhesiveness, can be obtained.

Said substrate layer can desirably be a powdery substrate layer, which is composed of a metal powder, or a bulk body. Here, in the substrate layer being a bulk body, metallic sintered bodies, which are formed by sintering a metal powder in another step being independent of the aforementioned sintering step, are included. When the substrate layer is adapted to a powdery substrate layer, it becomes possible to obtain a slide member by sintering a substrate and a sliding layer simultaneously. In addition, in the laminating step, when forming a powdery intermediate layer, which is composed of a metal powder, it becomes possible to obtain a slide member in which a substrate layer, an intermediate layer and a sliding layer are sintered simultaneously to form it.

Moreover, prior to said laminating step, it can desirably have a powder preparing step of preparing two members or more mixture powders in which the volume fractions between said resinous powder and said solid-lubricant powder at least differ; and, in said laminating step, said powdery sliding layer can desirably be formed by laminating said two members or more mixture powders sequentially so that a volume fraction of said solid-lubricant powder on its substrate-layer side becomes lower than on an opposite substrate-layer side, and thereby a functionally-gradient-material layer can be obtained with ease.

### BRIEF DESCRIPTION OF THE DRAWINGS

With reference to the following detailed description and the accompanying drawings, the present invention can be understood more profoundly. Hereinafter, the brief description of the drawings is done.

Fig. 1, Fig. 2 and Fig. 3 are cross-sectional diagrams for schematically illustrating an example of a slide member of the present invention. Fig. 4 is a cross-sectional diagram for schematically illustrating a sintering apparatus, which is used in plasma electrical discharge sintering. Moreover, Fig. 5 is a schematic diagram for illustrating a seizure test.

### BEST MODE FOR CARRYING OUT THE INVENTION

Hereinafter, the best mode for carrying out a slide member of the present invention and a production process of the present invention for a slide member will be explained, using Fig. 1, Fig. 2 and Fig. 3. Note that Fig. 1, Fig. 2 and Fig. 3 are cross-sectional diagrams for schematically illustrating an example of a slide member of the present invention.

[Slide Member]

A slide member of the present invention is a slide member, which has a substrate made of a metal; and a sliding layer of a resinous powder being sintered integrally on at least one of the surfaces of the substrate. And, the sliding layer includes a solid-lubricant powder.

The substrate is such that its size and configuration are not limited particularly, and can preferably be a bulk body, or a sintered body, which is composed of a metal powder being sintered integrally with the sliding layer. As described above, in the substrate being a bulk body, sintered bodies, which are composed of metal powders, not being those which are sintered integrally with the sliding layer, that is, sintered bodies, which are formed by means of sintering in advance before the resinous powder and the solid-lubricant powder are sintered, are included as well, in addition to metallic members, which are processed by means of casting, and the like.

Moreover, the substrate is such that it is not limited as far as it is made of a metal, and can preferably include at least one member of iron, aluminum, copper and magnesium. For example, when being an alloy, steels, aluminum alloys which include Mg, Cu, Zn, Si, Mn, and the like, and copper alloys which include Zn, Al, Sn, Mn, and so forth, and so on, are preferable.

When the substrate is a sintered body, which is composed of a metal powder which is sintered integrally with the sliding layer, the particle diameters of the metal powder can preferably be such that an average primary particle diameter is 10-200 µm, and further preferably 10-150 µm. When the particle diameters of the metal powder fall in the aforementioned ranges, the substrate, which has sufficient strength, can be obtained.

When the substrate is a bulk body, it is advisable that a surface treatment, such as plating treatments, thermal-spraying treatments, anodic-oxidation treatments, chemical-conversion treatments or rough-surface-forming treatments, can be done to the interface between it and the sliding layer. When these surface treatments are done, it is possible to improve the adhesiveness between the substrate and the sliding layer. Here, the plating treatments can be tin-plating treatments, Ni-plating treatments, Cu-plating treatments, and the like, for example. The thermal-spraying treatments can be Cu-thermal-spraying treatments, Al-Si-thermal-spraying treatments, and so forth, for instance. The anoidic-oxidation treatments, when the substrate is made of a material, which includes aluminummainly, can be alumite treatments, and so on, for example. The chemical-conversion treatments can be chromate treatments, non-chromate treatments, zinc phosphate treatments, and the like. The rough-surface-forming treatments can be shot blasting, etching, and so forth, for instance. Note that, by means of the aforementioned surface treatments, it is possible to form a later-described intermediate layer.

The sliding layer is composed of a resinous powder, which is sintered integrally on at least one of the surfaces of the substrate, and includes a solid-lubricant powder. Specifically, a raw material powder of the sliding layer (hereinafter being set forth as a raw material powder for the sliding layer) is composed of a resinous powder and a solid-lubricant powder at least, by means of sintering this raw material powder for the sliding layer, the sliding layer, which includes the sintered resinous powder and the solid lubricant powder, is formed. Here, it is advisable that at least one of the surfaces of the substrate can be a surface, which is equivalent to the sliding-surface side of the substrate. Note that the configuration of a sliding surface is such that it is not limited as far as it is a configuration, which fits for sliding, and can be a sliding surface, which comprises a curved surface, such as a spherical surface, in addition to a flat surface.

As described above, it has not been easy so far to obtain a laminated body, which comprises a metallic layer and a resinous layer whose adhesiveness is satisfactory to each other, by means of sintering. Whereas, the slide member of the present invention is such that, by means of having used a solid-lubricant powder in the sliding layer, the difference between the linear expansion coefficients of the substrate, which is made of a metal, and the sliding layer, which is made of a resin, becomes smaller, and accordingly it is possible to secure the adhesiveness between the substrate and the sliding layer. Further, because of the fact that a solid-lubricant powder exists in the sliding layer, the seizure resistance or wear resistance of an opposite substrate side (that is, being equivalent to a sliding-surface side) improves, and makes a slide member, which is suitable as a sliding portion. Moreover, since the sliding layer is such that, when heat is given to it by means of sintering, a resinous powder melts and then solidifies to form it, it is better in terms of the adhesiveness to the substrate than sliding layers which are formed by means of coating. Moreover, when it is sintered while being pressurized, the adhesiveness improves furthermore.

The sliding layer is such that its layer thickness is not limited in particular, but can preferably be 3-500 µm, especially preferably be 6-50 µm. When the layer thickness of the sliding layer falls in the aforementioned ranges, it makes a slide member, which has satisfactory adhesiveness and sliding characteristics.

Moreover, the sliding layer, in addition to a sliding layer 20 which is sintered in such a state that the distribution of a solid-lubricant powder is uniform as illustrated schematically in Fig. 1, can be a sliding layer which is sintered while making the amount of a solid-lubricant powder at least gradient. For example, as shown an example in Fig. 2, the sliding layer 20 can be a functionally-gradient-material layer in which the volume fraction of a solid-lubricant powder is lower on a substrate side (21) of the sliding layer than on an opposite substrate side (23). By means of adapting the sliding layer to a functionally-gradient-material layer, while holding the sliding characteristics on the opposite substrate side where the proportion of a solid-lubricant component is greater, it is possible to secure the adhesiveness between the substrate and the sliding layer on the substrate side where the proportion of a solid-lubricant component is less. This functionally-gradient-material layer can be a layer in which the proportion of a solid-lubricant powder changes continuously or stepwise (see Fig. 2) from a substrate side to an opposite substrate side. The details will be described later in the section of [Production Process for Slide Member].

The solid-lubricant powder is such that there is not any limitation on its amount; and, even when being an extremely small amount, can secure the adhesiveness between the substrate and the sliding layer; but it is preferable that, when a raw material powder for the sliding layer is taken as 100 Vol. %, the proportion of the solid-lubricant powder can be 20-80 Vol. %. When the proportion of the solid-lubricant powder falls within the aforementioned range, the adhesiveness between the substrate and the sliding layer becomes satisfactory.

Note that, in the sliding layer, it is advisable as well to make components other than the solid lubricant gradient; and it is advisable as well to make the proportion of a metal powder, which is composed of a metal or metallic oxide, or, among metals, especially, the proportion of the same kind of a metal powder as that of a metal, which constitutes the substrate or a later-described intermediate layer, gradient in the sliding layer. In this instance, the proportion of a metal powder is such that, by making it gradient so that it is higher on an substrate side of the slider layer than on an opposite substrate side, the adhesiveness between the substrate or intermediate layer and the sliding surface improves furthermore. Moreover, it is advisable as well to make the proportion of later-described respective additive agents gradient.

The solid-lubricant powders can be those, which have been used usually, such as a lamellar structural substance such as graphite or talc, a soft metal, such as Pb, Ag or Cu, and its compound, and a fluorine compound, such as polytetrafluoroethylene (PTFE). In particular, it can be at least one member of molybdenum disulfide powders, graphite powders and PTFE powders. Molybdenum disulfide is such that, in order to improve the wear resistance of the sliding layer, it is advisable to use those whose average primary particle diameter is 0.1-40 µm, preferably 1-10 µm. Graphite is such that, in order to make the adhesiveness inside the sliding layer satisfactory, it is advisable to use those whose average primary particle diameter is 0.1-10 µm, preferably 1-5 µm.

Moreover, the sliding layer can further contain either one of hard particles, an extreme-pressure agent, a surfactant, a working stabilizer agent and an oxidation prevention agent, or all the additive agents. That is, it is possible to use a powder of the additive agents as a raw material powder for the sliding layer. A powder of the additive agents is such that, as far as an appropriate amount, which depends on the required characteristics, is used, there is not any limitation on its proportion; but it is preferable that the proportion of a powdery additive agent can be 20 Vol. % or less when a raw material powder for the sliding layer is taken as 100 Vol. %; and it can especially preferably be included in an amount of 3-15 Vol. %. Moreover, the particle diameters of the additive agents are such that an average primary particle diameter can preferably be 0.1-10 µm, further preferably 0.3-3 µm.

Here, the hard particles can be alumina, silica, silicon carbide, silicon nitride, and the like, for instance. The extreme-pressure agent can be sulfur-containing metallic compounds, such as zinc sulfide (ZnS) or silver sulfide (Ag₂S), and so forth, for example. The surfactant can be fluorine-system surfactants, silicon-system surfactants, and so on, for instance.

The working stabilizer agent can be bifunctional-type working stabilizer agents, single-agent addition-type working stabilizer agents, and the like, for example. As for the bifuctional-type working stabilizer agents, "Sumilizer GM," a product name (chemical name: 2-tert-Butyl-6-(3-tert-butyl-2-hydroxy-5-methylbenzyl)-4-methylphenyl acrylate), produced by SUMITOMO KAGAKU KOGYO Co., Ltd., "Sumilizer GMS (F), " a product name (chemical name: 2-[1-(2-hydroxy-3,5-di-tert-pentylphenyl) ethyl]-4,6-di-tert-pentylphenyl acrylate), produced by SUMITOMO KAGAKU KOGYO Co., Ltd., and so forth, are available. As for the single-agent addition-type (SA-system) working stabilizer agents, "Sumilizer GP," a product name (chemical name: 6-[3-(3-t-Butyl-4-hydroxy-5-methylphenyl) propoxy]-2,4,8,10-tetra-t-butyldibenz [d,f] [1,3,2] dioxaphosphepin), produced by SUMITOMO KAGAKU KOGYO Co., Ltd., and so on, are available.

The oxidation prevention agent can be phenol-system primary oxidation prevention agents, organic sulfur-system secondary oxidation prevention agents, amine-system primary oxidation prevention agents, phosphite-system oxidation prevention agents, and the like, for instance. As for the phenol-system primary oxidation prevention agents, "Sumilizer MDP-S2," a product name (chemical name: 2'-Methylenebis(6-tert-butyl-4-methylphenol)), produced by SUMITOMO KAGAKU KOGYO Co., Ltd., "Sumilizer BBM-S," a product name (chemical name: 4,4'-Butylidenebis(6-tert-butyl-3-methylphenol)), produced by SUMITOMO KAGAKU KOGYO Co., Ltd., "Sumilizer WX-R WX-RA WX-RC," a product name (chemical name: 4,4'-Thio bis(6-tert-butyl-3-methylphenol)), produced by SUMITOMO KAGAKU KOGYO Co., Ltd., "Sumilizer NW (N), " a product name (chemical name: Alkylated bisphenol), "Sumilizer GA-80," a product name (chemical name: 3,9-Bis[2-[3-(3-tert-butyl-4-hydroxy-5-methylphenyl) propionyloxy]-1,1-dimethylethyl]-2,4,8,10-tetraoxaspiro [5·5] undecane), produced by SUMITOMO KAGAKU KOGYO Co., Ltd., and so forth, are available. As for the organic sulfur-system secondary oxidation prevention agents, "Sumilizer MB," a product name (chemical name: 2-Mercaptobenzimidazole), produced by SUMITOMO KAGAKU KOGYO Co., Ltd. , and so on, are available. As for the amine-system primary oxidation prevention agents, "Sumilizer 9A," a product name (chemical name: Alkylated diphenylamine), produced by SUMITOMO KAGAKU KOGYO Co., Ltd., and the like, are available. As for the phosphite-system oxidation prevention agents, "Adecastab PEP-36," a product name, produced by ASAHI DENKA KOGYO Co., Ltd., and so forth, are available.

The resinous powder is such that, as far as it is composed of a resin which can form the sliding layer by melting and then solidifying upon giving heat to it by means of sintering, there is not any limitation on its type particularly, but can preferably be a heat-resistant resinous powder which is composed of a heat-resistant resin not degradable by means of heating. Moreover, the particle diameters of the resinous powder are such that an average primary particle diameter can preferably be 1-200 µm, further preferably 10-120 µm. The slide member, which has the sliding layer obtained by sintering the resinous powder having particle diameters within the aforementioned ranges, exhibit suitable sliding characteristics.

Moreover, the resinous powder can preferably includes at least one member of polyamide imide resinous powders, polyimide resinous powders, polyether ether ketone resinous powders and polybenzimidasole resinous powders. Among these, since resins, like polyether ether ketone resins (PEEK resins), which are less likely to dissolve into solvents, cannot be coated, it has been difficult for them to form the sliding layer conventionally; however, using sintering makes it possible to form the sliding layer.

The slide member of the present invention, as schematically illustrated in Fig. 3, can preferably further have an intermediate layer 30, which intervenes between the substrate 10 and the sliding layer 20 and is composed of a metal differing from that of the substrate. Note that "a metal differing from that of the substrate" is such that, even when the intermediate layer and the substrate are the same kind of meal with each other, for example, they can differ in the compositions. By means of disposing an intermediate layer, even when such an instance occurs that the sliding layer is damaged during the slide member' s service, since it can keep sliding to adapt the intermediate layer to a sliding surface, the reliability as a slide member improves. When being an intermediate layer, which includes at least one member of copper and aluminum, it is effective furthermore.

The intermediate layer can preferably be an intermediate sintered-body layer, which is composed of a metal powder being sintered integrally with the substrate and the sliding layer. Moreover, it can be an intermediate layer, which is formed by performing a plating treatment, a thermal-spraying treatment, or the like, to a bulk-body substrate in advance. Moreover, although there is not any limitation on the layer thickness of the intermediate layer, it can preferably be 0.05-500 µm, further preferably be 0.1-300 µm. When the layer thickness falls in the aforementioned ranges, it makes a slide member, in which the adhesiveness to the sliding layer is satisfactory.

Note that the substrate can be a sliding component part for compressors. That is, the slide member of the present invention can be adapted to a slide member for compressors. For example, the slide member of the present invention can be used in a swash plate for swash plate-type compressors. Moreover, the slide member of the present invention can be used in a shoe for compressors. A "swash plate and shoe for swash plate-type compressors" are such that there arises the case that they slide with each other in a dry state without any lubricant in their initial period of operation. Even in the case that they slide in such a very severe dry state, it is desired that they do not cause seizure or wear. Hence, by using the slide member of the present invention, which is good in terms of the adhesiveness and which has high seizure resistance and wear resistance, for a swash plate or shoes for swash plate-type compressors, it is possible to satisfy the conditions, which are required for swash plate-type compressors.

In addition to those aforementioned, it can be used as well for a sliding bearing, which supports the driving shaft of a compressor. Moreover, it can be used for a rotary valve, which is supported axially to the driving shaft of a piston-type compressor integrally, and additionally which is supported pivotally to the housing of a piston compressor rotatably so as to rotate synchronously with the driving shaft to make the gas passage between the compression chamber and the inlet pressure region openable and closable; or for a piston for a piston-type compressor.

And, the slide member of the present invention can be obtained by means of a hereinafter-explained production process for a slide member.

[Production Process for Slide Member]

A production process of the present invention for a slide member has: a laminating step of forming a powdery sliding layer, which is composed of a resinous powder and a solid-lubricant powder at least, on at least one of the surfaces of a substrate layer, which is composed of a metal; and a sintering step of sintering the substrate layer with the powdery sliding layer integrally.

In the laminating step, it is possible to form a powdery sliding layer by disposing a raw material powder for the sliding layer, raw material powder which includes a resinous powder and a solid-lubricant powder at least, as a desired configuration on at least one of the surfaces of a substrate layer. Specifically, for instance, when charging a raw material powder for the sliding layer within a mold so as to be a desired thickness; then placing a substrate layer on it; and sintering them, a slide member, which has a sliding layer 20 on one of the opposite surfaces of a substrate 10 as illustrated in Fig. 1, can be obtained. Further, when charging a raw material powder for the sliding layer on a substrate layer within a mold so as to be a desired thickness; and sintering them, a slide member, which has a sliding layer on a metallic substrate's two surfaces disposed back-to-back, can be obtained. In this instance, when a substrate layer is a bulk body, it is advisable to dispose a metallic plate, or the like, whose size is accommodable within a mold, within the mold as a substrate layer. Moreover, when a substrate layer is a powdery substrate layer, which is composed of a metal powder, it is advisable to charge a metal powder within a mold so as to be a desired thickness. Note that, as described above, a substrate layer, which is a bulk body, is such that, in addition to metallic members, which are processed by means of casting, and the like, metallic sintered bodies, which are sintered in another step which differs from the aforementioned sintering step, are included as well.

When using a mold in the laminating step, by arbitrarily forming a powdery sliding layer's configuration by means of selecting the mold's configuration appropriately, it is possible as well to obtain a sliding layer, which possesses a sliding surface comprising a curved surface, such as a spherical surface, in addition to a flat surface. Further, when simultaneously sintering two or more layers (for example, a powdery substrate layer and a powdery sliding layer), which are composed of powders whose melting points differ, it is advisable to make a difference between the thermal conductivities by means of varying a mold's configuration or material quality so that the mold's temperature becomes appropriate temperatures for the sintering of the respective powders. Moreover, on the occasion of the sintering step, it is advisable to smooth the surface of a powder using a smoothing jig, and the like, or to form a formed body, which comprises a substrate layer and a powdery slide member, by means of compression molding, and so forth. In compression molding, by means of pressurizing in the thickness-wise direction of a powdery sliding layer, the adhesiveness of an obtained slide member improves.

Note that the aforementioned raw material powder for the sliding layer, raw material powder which is for forming a powdery sliding layer, is such that it is advisable to admix a resinous powder and a solid-lubricant powder at least by means of a ball mill, rod mill, a double-coated blender, a V-type mixer, and the like. In this instance, a metal powder or an additive agent, and so forth, too, can desirably be mixed all together with them.

By means of the laminating step, it is possible to make a solid-lubricant powder gradient as well. In a powder preparing step, by means of preparing two or more mixture powders, in which the volume fractions between a resinous powder and a solid-lubricant powder at least differ, in advance; and, in the laminating step, laminating the two or more mixture powders sequentially so that a volume fraction of the solid-lubricant powder on its substrate-layer side becomes lower than on an opposite substrate-layer side, the proportion of the solid-lubricant powder changes stepwise from the substrate side to the opposite substrate side. For example, as illustrated in Fig. 2, a slide member, which possesses sliding layers 21, 22 and 23 which are laminated sequentially on the surface of a substrate 10, can be obtained. In the slide member of Fig. 2, the sliding layers 21, 22 and 23 are such that the volume fraction of a solid-lubricant powder becomes greater in this order.

In this instance, it is advisable to vary the type of the resinous powder and solid-lubricant powder, or an additive agent, and the like, for each of the respective sliding layers. By means of this, it is possible to give characteristics, which are appropriate for the substrate-layer side and for the opposite substrate-layer side, respectively.

Moreover, when one would like to obtain a slide member in which the proportion of a solid-lubricant powder changes continuously from the substrate side to the opposite surface side, it is possible to bring about the continuous change by means of preparing a mixture powder, in which the volume fraction between a resinous powder and a solid-lubricant powder at least is changed more finely, for instance. Moreover, even a method makes it possible, method in which a solid-lubricant powder is fed into a mixing apparatus, in which a resinous powder is held in a certain fixed amount, in a certain fixed amount little by little; and simultaneously therewith a mixed raw material powder for a sliding layer is fed into a mold while carrying out admixing them at a sufficient rate in the mixing apparatus. Furthermore, by means of a centrifuge separation method, it is possible to change the volume fraction continuously. That is, a raw material powder for the sliding layer is put within a mold after mixing it uniformly; and subsequently the raw material powder for the sliding layer is separated centrifugally within the mold, thereby making the volume fraction gradient. Moreover, as another technique, it is possible as well to taper the volume fraction by means of moving a powder with a heavier weight downward continuously by means of giving a vibration to a uniform raw material powder for the sliding layer.

Further, it is advisable to make a powder, which is composed of a metal or a metallic oxide, or a metal powder, which is composed of a metal, among metals for forming a substrate layer or an intermediate layer especially, gradient in a powdery sliding layer. The method of making a metal powder gradient can be the same as the aforementioned methods of making a solid-lubricant powder gradient.

Moreover, the laminating step can desirably include a step of forming a powdery intermediate layer, which is composed of a metal powder differing from that of the substrate layer, between the substrate layer and the powdery sliding layer. By means of having a powdery intermediate layer, it becomes possible to simultaneously form at least a sliding layer and an intermediate layer by means sintering. For example, as schematically illustrated in Fig. 3, a sliding layer, which has an intermediate layer 30 on the surface of a substrate 10, and which further has a sliding layer 20 on the surface of the intermediate layer 30, can be obtained. Of course, the sliding layer 20 can be a functionally-gradient-material layer as well.

Alternatively, when a substrate layer is a bulk body, prior to the laminating step, it is advisable to have an intermediate-layer forming step of forming an intermediate layer, which is composed of a metal differing from that of the substrate layer, on the surface of the substrate layer, surface on which the powdery sliding layer is formed. As for a method of forming an intermediate layer, it is possible to name plating treatments or thermal-spraying treatments, and the like.

The sintering step is a step in which the substrate layer is sintered with the powdery sliding layer integrally at least. The powdery sliding layer is such that heat is given to it by means of the sintering step so that it is melted and then solidified, and thereby turns into a sliding layer. Moreover, when the substrate layer is a powdery substrate layer which is composed of a metal powder, the powdery sliding layer turns into a substrate, which is composed of a sintered body, by means of the sintering step. Further, when the intermediate layer is a layer which is composed of a metal powder, it turns into an intermediate layer, which is composed of a sintered body.

Therefore, in accordance with the production process of the present invention for a slide member, a slide member can be formed with a reduced number of steps by means of sintering the substrate layer with the powdery sliding layer, which is formed in the laminating step, integrally in the sintering step. Moreover, by means of adapting the substrate layer to a powdery substrate layer, it becomes possible to simultaneously sinter a substrate with a sliding layer to obtain a slide member. Further, by means of forming a powdery intermediate layer, which is composed of a metal powder, in the laminating step, it becomes possible to simultaneously sinter a substrate, an intermediate layer and a sliding layer to obtain a slide member.

Moreover, as for a sintering method, although it is possible to use conventional methods, such as hot pressing, especially preferable one is a sintering method in which the powdery sliding layer is discharge sintered while being pressurized with a mold; specifically, it can be a plasma electrical discharge sintering method. A plasma electrical discharge sintering method is a method in which a direct-current pulsating electric current is given between electrodes to carry out sintering, utilizing the discharge phenomenon between powders. Since powders are activated by means of discharge, an advantage is available in that they can be sintered at a lower temperature for a shorter period of time. Moreover, since it is sintered while being pressurized, a slide member, which is good in terms of the adhesiveness, is obtainable.

Note that, in the sintering step, there is not any limitation on the sintering conditions, and they can be conditions under which a resinous powder can be sintered satisfactorily. When substances, which are likely to be oxidized, are present in a raw material powder (a metal powder or a raw material powder for the sliding layer), it is desirable to sinter it in vacuum or in an inert gas atmosphere. Moreover, the sintering temperature can be selected appropriately depending on the types of raw material powders.

So far, although the embodiment modes of the slide member of the present invention and the production process for a slide member have been described, the slide member of the present invention and the production process for a slide member are not those which are limited to the above-described embodiment modes; but they can be carried out in various modes provided with such changes and modifications that one of ordinary skill in the art can carry out without departing from the spirit or scope of the present invention.

Hereinafter, an example of the slide member of the present invention and the production process of the present invention for a slide member will be explained using Fig. 4 and Fig. 5. Note that Fig. 4 is a cross-sectional diagram for schematically illustrating a plasma electrical discharge sintering apparatus, and Fig. 5 is an explanatory diagram of a seizure test.

In the present example, sintering was carried out using a plasma electrical discharge sintering method. A plasma discharge apparatus 4 (hereinafter, set forth as a "sintering apparatus" 4), as illustrated in Fig. 4, is such that an upper electrode 42 and a lower electrode 47 are disposed on a pressing apparatus 40, which is equipped with hydraulic devices 41, 46, and additionally an upper punch 43 and a lower punch 48 are disposed coaxially, and further is constituted of a vacuum chamber 44, an electric-power-source device and various control devices (not shown). And, powders (1' 2') or a metallic plate (1), which are put in a graphite mold 49 (not shown) with a 50-mm inside-diameter cylinder shape or a graphite mold 49' , are pressurized by means of the lower punch 43 and upper punch 48, and are then sintered by means of plasma discharge.

Note that, although the graphite mold 49 is a cylinder-shaped mold whose outside diameter (thickness) is uniform, the graphite mold 49' is such that the outside diameters differ between the upper portion and the lower portion as illustrated in Fig. 4. Accordingly, between the upper portion and lower portion of the graphite mold 49', the thermal conductivities differ.

Moreover, in the present example, an aluminum powder (average particle diameter: 30 µm), a copper powder (average particle diameter: 30 µm), and disk-shaped metallic plates (φ 50 mm, and thickness: 10 mm), which were composed of an aluminum alloy or a copper alloy, were prepared.

Further, mixture powders "A"-"E" (however, the powder E was composed of a resinous powder alone), in which a resinous powder was mixed with a solid-lubricant powder in the volume fractions set forth in Table 1 by means of a ball mill, were prepared. As for the resinous powder, either one of a polyamide imide (PAI) resinous powder (average primary particle diameter: 100 µm), a polyimide (PI) resinous powder (average primary particle diameter: 20 µm) and a polyether ether ketone (PEEK) resinous powder (average primary particle diameter: 100 µm) was used. Moreover, as for a solid lubricant, molybdenum disulfide (average primary particle diameter: 10 µm) and graphite (average primary particle diameter: 1 µm) were used in a volumetric ratio of 1 : 1.

**[TABLE 1]**

| Powder | Resinous Powder [Vol. %] (PAI, PI or PEEK) | Solid-lubricant | Powder [Vol. %] |
|---|---|---|---|
| | | Molybdenum Disulfide | Graphite |
| "A" | 70 | 15 | 15 |
| "B" | 60 | 20 | 20 |
| "C" | 50 | 25 | 25 |
| "D" | 25 | 37.5 | 37.5 |
| "E" | 100 | 0 | 0 |

(Making of Slide Members "a"-"f")

After charging the powder "C" in the graphite mold 49' of the sintering apparatus 4 from above, the surface of the powder "C" was smoothed by means of preliminary pressurizing by the upper punch 43 (it was an operation for arranging the configuration of the charged powder by pressurizing it with 20 MPa, but no plasma was generated in this instance) so that a powdery sliding layer 2' whose layer thickness was 500 µm was formed. Next, after charging a metal powder, either one of the aluminum powder or the copper powder, onto the smoothed powder "C, " the surface of the metal powder was smoothed by means of preliminary pressurizing by the upper punch 43 so that a substrate layer 1' whose layer thickness was 5 mm was formed. Note that the powder "C" was adapted so as to be positioned at the lower portion of the graphite mold 49' whose thickness was thicker; and the metal powder was adapted so as to be positioned at the upper portion of the graphite mold 49' whose thickness was thinner.

And, a direct-current pulsating electric current was applied to the substrate layer 1' and powdery sliding layer 2' in such a state that they were pressurized at 50 MPa, thereby carrying out plasma electrical discharge sintering. The sintering was such that slide members "a"-"f" were made by means of holding the temperature of the graphite mold 49' at 300-400 °C for 1-10 minutes.

Note that the types of the metal powders and resinous powders used for the slide members "a"-"f" are set forth in Table 2.

(Making of Slide Members "g"-"t")

Into the graphite mold 49 of the sintering apparatus 4, either one metallic plate of the aluminum alloy or the copper alloy was inserted from above. Next, after charging the powder "A" or the powder "C" onto the metallic plate, the surface of the mixture powder was smoothed by means of preliminary pressurizing by the upper punch 43 so that a first layer whose layer thickness was 500 µm was formed.

When forming a second layer on the first layer, after charging the powder "B" or the powder "C, " the surface of the mixture powder was smoothed by means of preliminary pressurizing by the upper punch 43 so that a second layer whose layer thickness was 500 µ m was formed.

Moreover, when forming a third layer on the second layer, after charging the powder "C," the surface of the mixture powder was smoothed by means of preliminary pressurizing by the upper punch 43 so that a third layer whose layer thickness was 500 µm was formed.

Furthermore, when forming a fourth layer on the third layer, after charging the powder "D," the surface of the mixture powder was smoothed by means of preliminary pressurizing by the upper punch 43 so that a fourth layer whose layer thickness was 500 µm was formed.

And, by means of sintering the metallic plate 1 and a powdery sliding layer 2' , which comprised the first layer, among the first layer-fourth layer, at least, in the same manner as the aforementioned slide members "a"-"f," slide members "g"-"t," which comprised a substrate 1 and a sliding layer 2, were made.

Note that the types of the metallic plates and resinous powders, which were used in the slide members "g"-"t, " and the types of the mixture powders, which were used for the first layer-fourth layer, are set forth in Table 2.

(Making of Slide Members "a'"-"f'")

Except that the powder "E" (not including any solid-lubricant powder) was employed instead of the powder "C," slide members "a"'-"f" were made in the same manner as the slide members "a"-"f." Note that the types of the metal powders and resinous powders, which were used for the slide members "a'"-"f'," are set forth in Table 2.

(Making of Slide Members "x," and "y")

After stirring a PAI varnish with a solid-lubricant powder well, they were fed through a three-piece roll mill, thereby preparing a coating composition. Note that the coating composition was prepared so as to make the proportions of the PAI powder and solid-lubricant powder identical with those of "C" in Table 1.

Next, the coating composition was coated onto the surface of a metallic plate 1 by means of spray coating method; after drying it, sintering was carried out at 200 °C for 1 hour, thereby making slide members "x" and "y," which comprised the metallic plate 1 and a sliding layer 2. Note that the layer thickness of the sliding layer 2 was 20 µm.

[Evaluation]

In order to confirm the effects of the slide member of the present invention, a seizure test was carried out with respect to the aforementioned respective slide members. Specifically, as illustrated in Fig. 5, on the top surface of shoes 6, which were fixed on a seating portion 7 and were composed of a bearing steel (SUJ2), the respective slide members, to which a rotary shaft 5 was fixed from the side of the substrate 1, were rotated about the shaft, thereby slidably contacting the sliding surface 2 with the top surface of the shoes 6.

And, the seizure test was carried out in such a manner that a sliding speed: 10 m/s; a load: 5,000 N; a testing time: 2 hours (7, 200 seconds) ; and under lubrication with a freezer oil. Moreover, the friction coefficients, which were after the testing load stabilized to 5, 000 N, were measured. The test results are set forth in Table 2.

**[Table 2]**

| | Type of Substrate | Sliding Layer | | | | | Test Result | | |
|---|---|---|---|---|---|---|---|---|---|
| | | Type of Resin | lst Layer | 2nd Layer | 3r Layer | 4th Layer | Friction Coefficient* | Seizure** | |
| Slide Member "a" | Aluminum Powder | PAI | "C" | | | | 0.008 | ⊚ | |
| Slide Member "b" | Aluminum Powder | PI | "C" | | | | 0.011 | ⊚ | |
| Slide Member "C" | Aluminum Powder | PEEK | "C" | | | | 0.010 | ⊚ | |
| Slide Member "d" | Copper Powder | PAI | "C" | | | | 0.014 | ⊚ | |
| Slide Member "e" | Copper Powder | PI | "C" | | | | 0.009 | ⊚ | |
| Slide Member "f" | Copper Powder | PEEK | "C" | | | | 0.010 | ⊚ | |
| Slide Member "g" | Aluminum Alloy | PAI | "A" | | | | 0.013 | ○ (2200) | |
| Slide Member "h" | Aluminum Alloy | PI | "A" | | | | 0.015 | ○ (1800) | |
| Slide Member "i" | Aluminum Alloy | PEEK | "A" | | | | 0.016 | ○ (2600) | |
| Slide Member "j" | Aluminum Alloy | PAI | "C" | | | | 0.012 | ○ (3600) | |
| Slide Member "k" | Aluminum Alloy | PAI | "A" | "C" | | | 0.010 0 | ⊚ | |
| Slide Member "1" | Aluminum Alloy | PAI | "A" | "B" | "C" | | 0.011 | ⊚ | |
| Slide Member "m" | Aluminum Alloy | PAI | "A" | "B" | "C" | "D" | 0.008 | ⊚ | |
| Slide Member "n" | Aluminum Alloy | PI | "C" | | | | 0.013 | ○ (3000) | |
| Slide Member "o" | Aluminum Alloy | PI | "A" | "B" | "C" | | 0.014 | ⊚ | |
| Slide Member "p" | Aluminum Alloy | PI | "A" | "B" | "C" | "D" | 0.010 | ⊚ | |
| Slide Member "q" | Aluminum Alloy | PEEK | "C" | | | | 0.011 | ⊚ | |
| Slide Member "r" | Aluminum Alloy | PEEK | "A" | "B" | "C" | | 0.010 | ⊚ | |
| Slide Member "s" | Aluminum Alloy | PEEK | "A" | "B" | "C" | "D" | 0.009 | ⊚ | |
| Slide Member "t" | Copper Alloy | PAI | "A" | "B" | "C" | | 0.011 | ⊚ | |
| Slide Member "a"' | Aluminum Powder | PAI | "E" | | | | - | - | Peeled off from Interface before Testing |
| Slide Member "b'" | Aluminum Powder | PI | "E" | | | | - | - | |
| Slide Member "c" | Aluminum Powder | PEEK | "E" | | | | - | - | |
| Slide Member "d"' | Copper Powder | PAI | "E" | | | | - | - | Peeled off from Interface before Testing |
| Slide Member "e'" | Copper Powder | PI | "E" | | | | - | - | |
| Slide Member "f'" | Copper Powder | PEEK | "E" | | | | - | - | |
| Slide Member "x" | Aluminum Alloy | PAI | "C" | | | | 0.011 | Δ (1000) | Coating |
| Slide Member "y" | Copper Alloy | PAI | "C" | | | | 0.012 | Δ (1200) | |

| | | | | | | | | | |
|---|---|---|---|---|---|---|---|---|---|
| * : Measuring the friction coefficients, which were after the testing load stabilized to 5,000 N. **: Those, in which no seizure occurred after the test, were regarded as ⊚. Those in parentheses specify the elapsed times when seizure occurred. | | | | | | | | | |

Note that, since the slide members "a'"-"c'," which did not include any solid-lubricant powder, were such that the sliding layer 2 was peeled off from the substrate 1 soon after the making of the slide members, the test was not carried out. Moreover, since the slide members "d'"-"f'," which similarly used the powder "E, " were such that the sliding layer 2 was peeled off from the substrate 1 before the testing load reached 5, 000 N (specifically, 1, 000-3, 000 N approximately), the test was not carried out subsequently thereafter.

All of the slide members "a"-"t" exhibited low friction resistance, and most of them were such that no seizure occurred after the 2-hour test. Moreover, in slide members "g," "h," "i," "j" and "n," although seizure occurred after 2,200 seconds, after 1,800 seconds, after 2,600 seconds, after 3,600 seconds and after 3,000 seconds, respectively, they were better in terms of the seizure resistance than the slide members "x" and "y," which were made by means of coating, were. This is because they are sintered while being pressurized so that the resinous powders melt and then solidify by means of sintering and additionally their adhesiveness to the substrate heightens by means of pressurizing.

Namely, the slide members "a"-"t," which have a metallic substrate, and a sliding layer of a resinous powder being sintered integrally on at least one of the surfaces of the substrate; and which include a solid-lubricant power in the sliding layer, are such that the adhesiveness between the substrate and the sliding layer is high, and have good sliding characteristics.

## Claims

1. A slide member having a substrate made of a metal; and a sliding layer a resinous powder being sintered integrally on at least one of the surfaces of the substrate,
the slide member being **characterized in that** it includes a solid-lubricant powder in said sliding layer.

2. The slide member set forth in claim 1, wherein at least said sliding layer is one which is discharge sintered while being pressurized with a mold.

3. The slide member set forth in claim 1, wherein said substrate is a bulk body, or a sintered body, which is composed of a metal powder being sintered integrally with said sliding layer.

4. The slide member set forth in claim 1, wherein said substrate includes at least one member of iron, aluminum, copper and magnesium.

5. The slide member set forth in claim 1, wherein said sliding layer is a functionally-gradient-material layer in which a volume fraction of said solid-lubricant powder on its substrate side is lower than on an opposite substrate side.

6. The slide member set forth in claim 5, wherein said functionally-gradient-material layer is a layer in which the proportion of said solid-lubricant powder changes continuously or stepwise from said substrate side to said opposite substrate side.

7. The slide member set forth in claim 1, wherein said solid-lubricant powder includes at least one member of a molybdenum disulfide powder, a graphite powder and a fluorine compound powder.

8. The slide member set forth in claim 1, wherein said resinous powder is a heat-resistant resinous powder composed of a heat-resistant resin.

9. The slide member set forth in claim 1, wherein said resinous powder includes at least one member of polyamide imide resinous powders, polyimide resinous powders and polyether ether ketone resinous powders.

10. The slide member set forth in claim 1 having an intermediate layer, which intervenes between said substrate and said sliding layer, and which is composed of a metal differing from that of the substrate.

11. The slide member set forth in claim 10, wherein said intermediate layer is an intermediate sintered-body layer, which is composed of a metal powder being sintered integrally with said substrate and said sliding layer.

12. The slide member set forth in claim 10, wherein said intermediate layer includes at least one member of copper and aluminum.

13. The slide member set forth in either one of claims 1-12, wherein said substrate is a sliding component part for a compressor.

14. A production process for a slide member being **characterized in that** it has:
a laminating step of forming a powdery sliding layer, which is composed of a resinous powder and a solid-lubricant powder at least, on at least one of the surfaces of a substrate layer, which is composed of a metal; and
a sintering step of sintering the substrate layer with the powdery sliding layer integrally.

15. The production process for a slide member set forth in claim 14, wherein, in said sintering step, at least said powdery sliding layer is discharge sintered while being pressurized with a mold.

16. The production process for a slide member set forth in claim 14, wherein said substrate layer is a powdery substrate layer, which is composed of a metal powder, or a bulk body.

17. The production process for a slide member set forth in claim 14, wherein: prior to said laminating step, it has a powder preparing step of preparing two members or more mixture powders in which the volume fractions between said resinous powder and said solid-lubricant powder at least differ; and
in said laminating step, said powdery sliding layer is formed by laminating said two members or more mixture powders sequentially so that a volume fraction of said solid-lubricant powder on its substrate-layer side becomes lower than on an opposite substrate-layer side.

18. The production process for a slide member set forth in claim 14, wherein said laminating step includes a step of forming a powdery intermediate layer, which is composed of a metal powder differing from that of the substrate layer, between said substrate layer and said powdery sliding layer.

19. The production process for a slide member set forth in claim 14, wherein: said substrate layer is a bulk body; and, prior to said laminating step, it has an intermediate-layer forming step of forming an intermediate layer, which is composed of a metal differing from that of the substrate layer, on the surface of the substrate layer, surface on which said powdery sliding layer is formed.
